

# United States Patent Office

3,645,902  
Patented Feb. 29, 1972

1

3,645,902

## FRICITION OR TRACTIVE DRIVE FLUID COMPRISING ADAMANTANES

Irl N. Duling, West Chester, Frederick P. Glazier, Thornton, and David S. Gates, Swarthmore, Pa., and Robert E. Moore, Wilmington, Del., assignors to Sun Oil Company, Philadelphia, Pa.  
No Drawing. Filed Nov. 14, 1969, Ser. No. 876,993  
The portion of the term of the patent subsequent to Aug. 3, 1988, has been disclaimed

Int. Cl. C09k 3/00

U.S. Cl. 252—73

11 Claims

### ABSTRACT OF THE DISCLOSURE

A friction or tractive drive comprises at least two relatively rotatable members in torque transmitting relationship, the tractive surfaces of the members having disposed thereon one or more tractants selected from at least one of the following groups (1) or (2):

- (1) a tractant comprising alkylated adamantane hydrocarbon having one adamantane nucleus per molecule with the  $C_3$ — $C_{20}$  alkyl moiety as a bridgehead substituent; and,
- (2) bis-type hydrocarbon product having two adamantane nuclei linked between bridgehead positions through the  $C_3$ — $C_{20}$  alkylene moiety.

### CROSS REFERENCES TO RELATED APPLICATIONS

The present application is copending with the following listed applications, all of which are assigned to the Sun Oil Company, to whom the present application is also assigned:

| Serial No.           | Filing date | Title                                                                                                                                                                 |
|----------------------|-------------|-----------------------------------------------------------------------------------------------------------------------------------------------------------------------|
| 621,443              | 3-8-67      | "Synthetic Lubricants From Low Molecular Weight Olefins"—Richard S. Stearns, Irl N. Duling and David S. Gates.                                                        |
| 679,801 <sup>1</sup> | 11-1-67     | "Traction Drive Transmission Containing Adamantane Compounds as Lubricant"—Irl N. Duling, Frederick P. Glazier, David S. Gates and Robert E. Moore.                   |
| 679,833              | 11-1-67     | "Traction Drive Transmission Containing Napthenes, Branched Paraffins, or Blends of Napthenes and Branched Paraffins as Lubricant"—Irl N. Duling and David S. Gates.  |
| 679,834              | 11-1-67     | "Blending Branched Paraffin Fluids for Use in Traction Drive Transmission"—Irl N. Duling, David S. Gates and Thomas D. Newingham.                                     |
| 784,487              | 12-17-68    | "Conversion of Adamantane Hydrocarbons to Monooleins"—Robert E. Moore.                                                                                                |
| 794,844              | 1-24-69     | "Friction Drive Fluid"—Irl N. Duling, and Frederick P. Glazier.                                                                                                       |
| 812,516              | 2-19-69     | "Catalytic Hydrofinishing of Petroleum Distillates in the Lubricating Oil Boiling Range"—Ivor W. Mills, Glenn R. Dimeler, Merritt C. Kirk, Jr. and Albert T. Olenzak. |
| 823,138              | 5-8-69      | "Reaction for Linking Nuclei of Adamantane Hydrocarbons"—Abraham Schneider.                                                                                           |
| 850,717              | 8-18-69     | "Hydrorefined Lube Oil and Process of Manufacture"—Ivor W. Mills and Glenn R. Dimeler.                                                                                |
| 851,488              | 8-19-69     | "Reaction of Alkyladamantane Compounds to Form Products Having Two Linked Adamantane Nuclei"—Robert E. Moore and Abraham Schneider.                                   |
| 3,256 <sup>1</sup>   | 8-19-69     | "Friction or Tractive Drive Fluid"—Irl N. Duling, Frederick P. Glazier, David S. Gates and Robert E. Moore.                                                           |
| 877,004              | 11-14-69    | "Reaction of Normal Paraffins with Adamantane Compounds"—Robert E. Moore.                                                                                             |

<sup>1</sup> The present application is a continuation-in-part of these two applications.

The disclosure of all of the above-referred to applications is hereby incorporated herein by reference, particularly as to disclosure therein directed to the preparation of compounds containing one or more adamantane nuclei, to the preparation of hydrogenated petroleum oils, saturated cyclic hydrocarbon oils or branched chain acyclic hydrocarbon oils and to the blending or hydrocarbon components to produce traction fluids.

Application Ser. No. 851,488 is now abandoned; however, a continuation-in-part-thereof Ser. No. 56,680, was filed July 27, 1970. Another related application is Ser. No. 679,851, filed Nov. 11, 1967.

### BACKGROUND OF THE INVENTION

Friction or traction drive systems for the transmission of power and testing equipment for determination of the traction coefficient have been described in numerous prior art references. See, for example, the following:

2

- (1) Rounds, F. G., U.S. Pat. No. 3,394,603, dated July 30, 1968
- (2) Hamman, W. C. and Schisla, R. M., U.S. Pat. No. 3,411,369, dated Nov. 19, 1968
- (3) Hamman, W. C. and Schisla, R. M., U.S. Pat. No. 3,440,894, dated Apr. 29, 1969
- (4) Rounds, F. G., J. of Chem. and Eng. Data, vol. 5, No. 4, pp. 499—507 (October 1960)
- (5) Hewko, Rounds and Scott, Proceeding of the Symposium on Rolling Contact Phenomena, pp. 157—185, Elsevier Publishing Co., Amsterdam (1962)
- (6) Almen, J. O. U.S. Pat. No. 2,045,555
- (7) Hewko, Roller Traction Drive Unit for Extremely Quiet Power Transmission, AIAA Paper 67-429

15 Applications of Irl N. Duling, David S. Gates and Robert E. Moore, Ser. No. 679,801, filed Nov. 1, 1967 and Ser. No. 3,256, filed Aug. 19, 1969, are directed to the use of adamantane compounds as traction fluids or as components of traction fluids.

### SUMMARY OF THE INVENTION

A friction or tractive drive comprising at least two relatively rotatable members in torque transmitting relationship, the tractive surfaces of said members having disposed thereon a tractant comprising at least one member selected from at least one of the following groups (1) or (2):

- (1) alkylated adamantane hydrocarbon having one adamantane nucleus per molecule with the  $C_3$ — $C_{20}$  alkyl moiety as a bridgehead substituent, more preferably, alkyladamantane hydrocarbon material represented by  $QX$  wherein  $Q$  is a  $C_{12}$ — $C_{14}$  alkyladamantyl group with a bridgehead valence selected from dimethyladamantyl, trimethyladamantyl, ethyladamantyl, methylethylada-

30 mantyl and dimethylethyladamantyl and  $X$  is a  $C_4$ — $C_{20}$  alkyl group terminally attached at said valence and at least predominantly of the structure



60 wherein  $n$  is an integer of 1 to 17, and

- (2) bis-type hydrocarbon product having two adamantane nuclei linked between bridgehead positions through the  $C_3$ — $C_{20}$  alkylene moiety.

65 These adamantanes can be obtained by means disclosed in the previously referred to application of Robert E. Moore, filed of even date with the present application.

70 As can be seen from the previously cited references, special properties are required of the traction fluids used in friction drive systems. One desired property is a high

coefficient of traction as measured for example, by the test procedure described in reference (4) supra. As shown therein, most materials have traction coefficients (measured at 200° F., 400,000 p.s.i. and at a bearing speed of 600 ft./min.) less than 0.06, with the values for hydrocarbons usually falling in the range of 0.03-0.05. In comparison, alkyladamantanes and bis-type products of the previously-referred to application of Moore and Schneider (including the ethers as well as the hydrocarbon dimers) generally have traction coefficients measured in this manner in the neighborhood of 0.06 or higher. They are thus particularly valuable as traction fluids or as additives for improving the traction coefficients of known types of traction fluid compositions. The products which are liquid at room temperature and atmospheric pressure are preferred for this purpose, but those which are normally solids also can be used to the extent that they are substantially soluble in the base fluid at the temperatures and pressures at which it is required to operate in the friction drive system.

Especially useful traction fluids comprise from 5-95% by volume of one or more such alkyladamantanes or bis-type hydrocarbons of the Moore application and from 95-5% of an acyclic branched chain fluid polymer of a C<sub>3</sub>-C<sub>8</sub> monoolefin, said fluid polymer having, preferably, a SUS viscosity at 100° F. in the range of 20-20,000 SUS, and, more preferably, at ASTM viscosity index in the range of 30-160. Preferably, the final, blended traction fluid has an SUS viscosity at 100° F. in the range of 30-15,000.

#### FURTHER DESCRIPTION

As is disclosed in the above-referred to copending application of Robert E. Moore saturated adamantanane hydrocarbons of the C<sub>10</sub>-C<sub>19</sub> range having 0-3 alkyl substituents and/or their corresponding adamantanols are reacted with n-paraffins of the C<sub>3</sub>-C<sub>20</sub> range by contacting a mixture of such reactants with sulfuric acid having a strength of 96-102% H<sub>2</sub>SO<sub>4</sub> equivalent at a temperature between the freezing point of the acid and 100° C., more preferably 10-75° C. This causes a C<sub>3</sub>-C<sub>20</sub> alkyl or alkylene moiety, derived from and having the same number of carbon atoms as the n-paraffin used, to become attached to the adamantanane nucleus. As a result, two types of products are obtained: (1) alkylated adamantanane hydrocarbon having one adamantanane nucleus per molecule with the C<sub>3</sub>-C<sub>20</sub> alkyl moiety as a bridgehead substituent; and (2) bis-type hydrocarbon product having two adamantanane nuclei linked between bridgehead positions through the C<sub>3</sub>-C<sub>20</sub> alkylene moiety. Generally, both types of product can be produced in substantial yields. They can be recovered in admixture with each other, such a mixture being particularly useful as a tractant or a component of a tractant for a friction or tractive drive.

Preferred products for use as a tractant or in tractant blends are those made from C<sub>5</sub>-C<sub>8</sub> n-paraffins and C<sub>12</sub>-C<sub>14</sub> alkyladamantanes or alkyladamantanols in which the alkyl substituents are methyl and/or ethyl.

Preferred adamantanane reactant material for producing tractants by the process are the alkyladamantanane hydrocarbons of the C<sub>12</sub>-C<sub>19</sub> range having one, two or three alkyl substituents, or their monoools. The presence of alkyl groups on the nucleus of the feed material usually tends to reduce the solidification point of the resulting products and give them wider utility in traction fluid applications. The most preferred alkyladamantanane reactant compounds are the hydrocarbons of the C<sub>12</sub>-C<sub>14</sub> range and particularly the following: dimethyladamantanane, trimethyladamantanane, ethyladamantanane, methylethyladamantanane and dimethylethyladamantanane. Some specific examples of these and other hydrocarbons that can be used are as follows: adamantanane; 1 - methyladamantanane; 2 - methyladamantanane; 1,2-, 1,3- and 1,4-dimethyladamantanane; 1- and 2-ethyladamantanane; 1 - ethyl - 3 - methyladamantanane; 1 - ethyl - 4 - methyladamantanane; 1,2,4-, 1,2,5-, 1,3,4- and 1,3,6 - trimethyladamantanane; 1 - ethyl - 2,4-dimethyl-

adamantanane; and 1 - ethyl - 3,6 - dimethyladamantanane. Illustrative examples of other starting hydrocarbons containing higher alkyl groups are: 1- and 2-butyladamantanane; 1 - methyl - 3 - propyladamantanane; 1,3-dimethyl-5 - butyladamantanane; 1 - ethyl - 2 - methyl - 5-hexyladamantanane; 1 - pentyl - 4 - methyladamantanane; 1,3-disobutyladamantanane; n-hexyladamantanane; n-nonyladamantanane; and the like.

Any adamantanol corresponding to the hydrocarbons as above defined is also suitable as reactant material. The hydroxy group can be located at either a bridgehead or nonbridgehead position on the nucleus. Substantially the same results will be obtained regardless of the original position of the —OH radical on the nucleus, inasmuch as immediate isomerization of the —OH to an unsubstituted bridgehead position on the nucleus occurs in the presence of the strong sulfuric acid used in the process.

The other reactant in the process is a normal paraffin hydrocarbon of the C<sub>3</sub>-C<sub>20</sub> range. Whereas the n-paraffins

themselves in the presence of strong sulfuric acid are normally inert, they become quite reactive when the adamantanane compound is also present and can readily function as an agent for alkylating the adamantanane nucleus. Any normal paraffin ranging from propane to eicosane or any mixture of these n-paraffins can be used in the process. When a higher molecular weight n-paraffin of the group herein defined is used, a reaction temperature in the upper part of the herein specified range preferably is employed. For preparing material for use in traction fluid compositions, n-paraffins of the C<sub>4</sub>-C<sub>8</sub> range are particularly suitable reactants. One useful mixture of C<sub>4</sub>-C<sub>8</sub> n-paraffins is obtained by separation of n-paraffins from "virgin" or "straight-run" gasoline by means of molecular sieve adsorbents.

Reaction of the adamantanane hydrocarbon or monoool feed material with the n-paraffin in accordance with the invention is effected by contacting a mixture of these reactants with strong sulfuric acid. The molar ratio of the adamantanane compound to the n-paraffin can vary widely in the reaction mixture but usually will be in the range of 3:1 to 1:10. The ratio of acid to reactants can vary widely. Generally a volume excess of the acid relative to the reactants should be used and a volume ratio thereof in the range of 1:1 to 20:1 typically is employed. The mixture normally is an emulsion of acid and hydrocarbon phases, and the reaction takes place in the acid phase. The sulfuric acid should have a strength in the range of 96-102% H<sub>2</sub>SO<sub>4</sub> equivalent by weight and more preferably 97-101% H<sub>2</sub>SO<sub>4</sub>. The reaction temperature can be from just above the freezing point of the acid used to about 100° C. and usually is in the range of 10-75° C. When a lower alkane such as propane or butane is used as reactant, the reaction is conducted under sufficient pressure to maintain a substantial concentration of the alkane in the liquid phase.

#### EXAMPLES

As a specific illustration of the invention, the reaction of n-pentane with 1,3-dimethyladamantanane (DMA) is considered. This reaction is effected, for example, by contacting a mixture of DMA and n-pentane in a molar ratio of 1:2 with sulfuric acid having a strength of 100% H<sub>2</sub>SO<sub>4</sub> at 50° C. for 10 hours. The acid and hydrocarbon layers are separated, the hydrocarbon layer is washed with water or aqueous alkali to remove residual acid, and the hydrocarbon material is then fractionally distilled to recover the products. The alkyladamantanane product upon analysis is found to be composed mainly of the following (hydrogen atoms omitted for convenience):



Specifically this product is 1,3-dimethyl-5-(3-methylbutyl) adamantanane. Smaller amounts of isomeric product with

the methyl branch in the  $C_5$  alkyl substituent positioned closer to the adamantane nucleus may also be produced, but the predominant isomer formed is the one shown. No isomer having an n-pentyl group is detected. A higher boiling bis-type product is also obtained and the major part thereof is found to correspond to the following structure:



This compound specifically is 1,4-bis(3,5-dimethyladamantyl-1)-4-methylbutane. A minor amount of product which boils closely to this compound and appears to be 15 isomeric thereto generally is also produced.

A blend is made of 60 volume percent of the above-referred to isomer mixture and 40% of a substantially fully hydrogenated polybutene polymer. The traction coefficient (by the Rounds method) at 600 ft./min., 400,000 p.s.i. and 200° F. is 0.059. This 60/40 blend also has good oxidation stability compared with the hydrogenated polybutene, good fluid properties and a greatly decreased tendency to foam when used in a traction drive.

Similarly, when the feed paraffin in the above reaction is n-hexane instead of n-pentane, the product of the reaction comprises a mixture of 1,3-dimethyl-5-(4-methylpentyl)adamantane and 1,4 - bis(3,5-dimethyladamantyl-1)-5-methylpentane. The traction coefficients (at 60 ft./min., 400,000 p.s.i. and 200° F.) for these individual compounds are 0.060 and 0.061, respectively.

When the feed paraffin is n-butane, the product of the reaction comprises a mixture of 1,3-dimethyl-5-(2-methylpropyl)adamantane and 1,4 - bis(3,5-dimethyladamantyl-1)-3-methylpropane. This mixture and these individual components are good tractants, especially when blended with  $C_3$ - $C_8$  polymer oils (or hydrogenated  $C_3$ - $C_8$  polymer oils).

When a monool of DMA is used instead of the hydrocarbon, the same two hydrocarbon compounds as shown above are again obtained as the major products regardless of the original position of the hydroxy group on the nucleus. However, the reaction tends to proceed to completion more rapidly when the starting adamantane compound is a monool instead of the hydrocarbon.

It is characteristic of the main products of the Moore process that, for any of the n-paraffins except propane, the alkyl and alkylene groups derived from the n-paraffin each will have a single methyl branch. Furthermore the methyl substituent in the alkyl group will be attached mainly to the second carbon adjacent the unattached end of the chain, while that in the alkylene group will be attached mainly to an alpha carbon atom in the chain. In other words, the alkyl and alkylene groups in the main products of the reaction will conform, respectively, to the following arrangements:



When n-paraffins of the  $C_4$ - $C_8$  range are used as reactant,  $n$  and  $m$  in these formulas would be integers which are, respectively, 1 to 5 and 2 to 6. The presence of the methyl substituents in the alkyl and alkylene moieties of the reaction products is beneficial for utilization of the products as components of traction fluids, as the methyl branches tend to prevent crystallization and lower the solidification or pour points of the products.

Both types of alkylation products are usually obtained from the present reaction, but the proportions thereof can vary considerably depending upon the particular reactants and conditions selected. As a general rule, formation of the bis-type product relative to the alkyladamantane is favored by higher acid concentrations and higher tem-

peratures and by using a monool reaction instead of the adamantane hydrocarbons as feed material.

From the present process when utilizing one or more  $C_{12}$ - $C_{14}$  alkyladamantanes or alkyladamantanols and one or more  $C_4$ - $C_{20}$  n-paraffins, a particularly desirable mixture can be recovered composed of a combination of the two types of alkylated adamantane products as above described. This constitutes a novel composition which has outstanding utility as a component of traction fluids. Both 10 types of reaction products have unusually high traction coefficients as compared to most hydrocarbons. Also the fact that the mixture involves a plurality of hydrocarbons containing adamantane nuclei is advantageous, since the pour point is reduced and an intermediate viscosity level desirable for various traction system applications is secured.

This novel composition suitable as a traction fluid component can be defined as a mixture of hydrocarbons containing adamantane nuclei and composed of a combination of the following:

(1) alkyladamantane hydrocarbon material represented by  $QX$  wherein  $Q$  is a  $C_{12}$ - $C_{14}$  alkyladamantyl group with a bridgehead valence selected from dimethyladamantyl, trimethyladamantyl, ethyladamantyl, methyl-ethyladamantyl and dimethyl-ethyladamantyl and  $X$  is a  $C_4$ - $C_{20}$  alkyl group terminally attached at said valence and at least predominantly of the structure



wherein  $n$  is an integer of 1 to 17, and

(2) bis-type alkyladamantane material represented by  $QZQ$  wherein  $Q$  is as previously specified and  $Z$  is a  $C_4$ - $C_{20}$  alkylene group linking the  $Q$ 's between bridgehead positions and at least predominantly of the structure



wherein  $m$  is an integer from 2 to 18.

Many of the alkyladamantane and bis-type products produced by the Moore process are oils at room temperature and exhibit unusually high traction coefficients. They are particularly useful as components of traction fluids for use in friction drive or toric transmission systems. Some of the products (in pure form) have sufficient symmetry to be relatively high melting solids, and these can have utility as components in traction fluids containing a solubilizing agent, such as a fluid naphthene hydrocarbon, or a fluid branched paraffin or olefin acyclic hydrocarbons or a mixture of naphthene and acrylic hydrocarbons.

Suitable components for blending with the alkyladamantanes of the Moore application, in order to produce improved, blended traction fluids are those oils prepared by polymerization of olefins, hydrogenated polyolefin oils (particularly when substantially free of olefinic unsaturation), hydrogenated hydrocarbon oils and saturated cyclic and acyclic hydrocarbons described in the above-referred to copending patent applications Ser. Nos. 679,801; 679,833, 679,834; 679,851 and 794,844. Particularly useful fluids for such blending are (1) hydrogenated naphthenic or paraffinic oils containing no more than 1 weight percent of "gel" aromatics, (2)  $C_{12}$ - $C_{70}$  organic liquids having at least one saturated ring and having a coefficient of traction of at least 0.06 as defined in U.S. Pat. No. 3,440,894, (3) a fused saturated component having from 2 to 9 fused rings and a total carbon content of from about 9 to about 60 as described in U.S. Pat. No. 3,411,369, (4) liquid hydrocarbon having an acyclic structure with at least three quaternary carbon atoms, as described in U.S.

Pat. No. 3,440,894, (5) members of groups (2) to (4) inclusive wherein up to 8 carbon atoms are replaced by atoms selected from the group consisting of oxygen, nitrogen, phosphorous and silicone (e.g., see U.S. Pat. No. 3,411,369 and U.S. Pat. No. 3,440,894). Fluorinated compounds corresponding to any of the above-referred to adamantane compounds wherein from 1-all of the hydrogen in the hydrocarbon has been replaced by fluorine are also useful as traction fluids or as components of traction fluids, particularly in blended fluids with hydrogenated olefin polymers.

The invention claimed is:

1. In a friction or tractive drive comprising at least two relatively rotatable members in torque transmitting relationship and a traction fluid, the improvement wherein, the tractive surfaces of said members have disposed thereon a traction fluid consisting essentially of a member selected from the following groups (1) or (2):

(1) alkyladamantane hydrocarbon material represented by QX wherein Q is a  $C_{12}$ – $C_{14}$  alkyladamantyl group with a bridgehead valence selected from dimethyladamantyl, trimethyladamantyl, ethyladamantyl, methylethyladamantyl and dimethylethyladamantyl and —X— is a  $C_4$ – $C_{20}$  alkyl group terminally attached at said valence and at least predominantly of the structure



wherein  $n$  is an integer of 1 to 17, and

(2) bis-type hydrocarbon product having two adamantane nuclei linked between bridgehead positions through a  $C_4$ – $C_{20}$  alkylene moiety having the same number of carbon atoms and skeletal structure as —X—.

2. A friction or tractive drive according to claim 1 and comprising a power input member and a power output member in tractive rolling contact relationship and a fluid film between said members, said fluid film consisting essentially of at least one member from said group (1) or said group (2) or mixtures thereof.

3. A drive according to claim 2 wherein said fluid film additionally contains from 95–5% by volume of a fully hydrogenated polymer of  $C_3$ – $C_8$  olefin.

4. A drive according to claim 1 wherein said alkyladamantane is selected from the following group:

1,3-dimethyl-5-(3-methylbutyl)adamantane  
1,3-dimethyl-5-(2-methylpropyl)adamantane  
1,3-dimethyl-5-(4-methylpentyl)adamantane  
1,4-bis(3,5-dimethyladamantyl-1)-4-methylbutane  
1,4-bis(3,5-dimethyladamantyl-1)-3-methylpropane  
1,4-bis(3,5-dimethyladamantyl-1)-5-methylpentane

5. A drive according to claim 2 wherein said tractant consists essentially of a mixture of:

(1) alkyladamantane hydrocarbon material represented by QX wherein Q is a  $C_{12}$ – $C_{14}$  alkyladamantyl group with a bridgehead valence selected from dimethyladamantyl, trimethyladamantyl, ethyladamantyl, methylethyladamantyl and dimethylethyladamantyl and X is a  $C_4$ – $C_8$  alkyl group terminally attached at said valence and at least predominantly of the structure



wherein  $n$  is an integer of 1 to 5, and

5 (2) bis-type alkyladamantane material represented QZQ wherein Q is as previously specified and Z is a  $C_4$ – $C_{20}$  alkylene group linking the Q's between bridgehead positions and at least predominantly of the structure



10 wherein  $m$  is an integer from 2 to 18.

6. A drive according to claim 5 wherein group (2), —Z— is a  $C_4$ – $C_8$  alkylene group and  $m$  is an integer from 2 to 6.

15 7. A drive according to claim 3 wherein said tractant consists essentially of from 5–95% by volume of one or more of said alkyladamantane isomers of group (1) and from 95–5% of an acyclic branched chain fluid polymer of a  $C_3$ – $C_8$  monoolefin, said fluid polymer having an SUS viscosity at 100° F. in the range of 20–20,000 SUS and an ASTM viscosity index in the range of 30 to 160.

20 8. A drive according to claim 7 wherein said tractant has a viscosity in the range of 30–15,000 SUS at 100° F.

25 9. A tractant composition consisting essentially of at least one member from the following groups (1) or (2):

30 (1) alkyladamantane hydrocarbon material represented by QX wherein Q is a  $C_{12}$ – $C_{14}$  alkyladamantyl group with a bridgehead valence selected from dimethyladamantyl, trimethyladamantyl, ethyladamantyl, methylethyladamantyl and dimethylethyladamantyl and X is a  $C_4$ – $C_{20}$  alkyl group terminally attached at said valence and at least predominantly of the structure



35 wherein  $n$  is an integer of 1 to 17, and

(2) bis-type hydrocarbon product having two adamantane nuclei linked between bridgehead positions through the  $C_4$ – $C_{20}$  alkylene moiety and from 95–5% by volume of a fully hydrogenated polymer of  $C_3$ – $C_8$  olefin.

40 10. A tractant composition according to claim 9 wherein said member from group (1) is

1,3-dimethyl-5-(3-methylbutyl)adamantane  
1,3-dimethyl-5-(2-methylpropyl)adamantane  
1,3-dimethyl-5-(4-methylpentyl)adamantane  
1,4-bis(3,5-dimethyladamantyl-1)-4-methylbutane  
1,4-bis(3,5-dimethyladamantyl-1)-3-methylpropane  
1,4-bis(3,5-dimethyladamantyl-1)-5-methylpentane

45 11. A tractant composition according to claim 9 wherein said member from group (1) consists of:

50 (1) alkyladamantane hydrocarbon material represented by QX wherein Q is a  $C_{12}$ – $C_{14}$  alkyladamantyl group with a bridgehead valence selected from dimethyladamantyl, trimethyladamantyl, ethyladamantyl, methylethyladamantyl and dimethylethyladamantyl and X is a  $C_4$ – $C_8$  alkyl group terminally attached at said valence and at least predominantly of the structure



55 wherein  $n$  is an integer of 1 to 5,

and said members from group (2) consist of:

(2) bis-type alkyladamantane material represented by QZQ wherein Q is as previously specified and Z is a C<sub>4</sub>-C<sub>20</sub> alkylene group linking the Q's between bridgehead positions and at least predominantly of

|           |         |                 |       |          |
|-----------|---------|-----------------|-------|----------|
| 3,203,186 | 8/1965  | Sheppard        | ----- | 60-54.5  |
| 3,208,946 | 9/1965  | Anderson et al. | ----- | 252-59   |
| 3,285,851 | 11/1966 | Dyer            | ----- | 252-32.5 |
| 3,382,288 | 5/1968  | Schneider       | ----- | 260-666  |
| 3,398,165 | 8/1968  | Duling et al.   | ----- | 260-410  |
| 3,411,369 | 11/1968 | Hammann et al.  | ----- | 74-200   |
| 3,440,894 | 4/1969  | Hammann et al.  | ----- | 74-200   |



wherein *m* is an integer from 2 to 18.

LEON D. ROSDOL, Primary Examiner

10 H. A. PITLICK, Assistant Examiner

U.S. Cl. X.R.

References Cited

UNITED STATES PATENTS

- |           |        |                   |       |         |    |
|-----------|--------|-------------------|-------|---------|----|
| 2,789,091 | 4/1957 | Crookshank et al. | ----- | 252-42  | 15 |
| 3,128,316 | 4/1964 | Schneider         | ----- | 260-666 |    |

74-200; 208-18, 19; 252-59; 260-666 M